

# UNITED STATES PATENT OFFICE.

HUGO SCHULTE-STEINBERG, OF DUEREN BEI STOCKUM, KREIS BOCHUM,  
GERMANY.

## PROCESS OF MANUFACTURING BRIQUETS OF ORE, &c.

No. 833,005.

Specification of Letters Patent.

Patented Oct. 9, 1906.

Application filed February 25, 1904. Serial No. 195,204.

*To all whom it may concern:*

Be it known that I, HUGO SCHULTE-STEINBERG, of Dueren bei Stockum, Kreis Bochum, Westphalia, Germany, have invented certain new and useful Improvements in Processes of Manufacturing Briquets Suitable to be Furnaced of any Metalliferous Refuse or Waste or Rotten Ores, of which the following is a specification.

10 The present invention relates to a process of manufacturing briquets for smelting and blast furnaces to reduce any metalliferous refuse or rotten ores, and has for its object, first, to permit the metallurgical utilization 15 of furnace refuse, rotten ores, or other metalliferous materials hitherto regarded as of no value, and, second, to dispense with the use of lime, hydraulic cement, or similar ingredients hitherto employed as binders in the manufacture 20 of similar briquets.

In the different methods heretofore employed for the manufacture of such briquets lime, hydraulic cement, or similar matters were used as binders. These, however, impair 25 the process of smelting and are unfit for the production of briquets with a certain degree of porosity, which is very desirable. The agglomeration of fine particles of ore has also been effected by mixing to it finely-commi- 30 nuted ordinary slag and by subsequently applying heat in order to fuse the slag so that the latter acts as a binder for the ore particles. A briquet obtained in this way is a good commercial article, but is expensive on 35 account of the fuel expended for fusing the slag. It is evident that a binder as a substitute for limestone, &c., consisting of furnace-slag, should give excellent results.

The binding power of ground or otherwise 40 comminuted or granular slag after a treatment with high-pressure steam in a closed cylinder or retort is well known, and such binder has been used to manufacture artificial sandstone for building purposes, having 45 a high degree of durability. The use of the same binder for making briquets for smelting purposes recommended itself; but certain difficulties had to be overcome, for the briquets require a certain degree of hardness, so 50 as to stand the handling, transportation, and to retain their shape in the furnace, while, on the other hand, a high degree of porosity, to be obtained by more or less sacrificing the hard-

ness, is very desirable, so that for the chemical actions in all the zones of the furnace the fine particles are easily and everywhere fully exposed. In using too much of the binder 55 briquets are obtained which, like the artificial sandstone above referred to, are very hard and useless for metallurgical reduction, 60 because they form lumps in the furnace which are inaccessible to the chemical reactions.

In using the binder in too small quantities the briquets obtained are insufficient for handling, fall into powder, and the small particles of ore, dust, &c., are compelled to follow the blast, leading to obstructions in the furnace, to explosions, and other irregularities. After many experiments I have found 70 that about ten per cent. is the most suitable quantity of the binder to be used with the metalliferous refuse in order to obtain briquets being sufficiently hard and having a suitable porosity.

75 In preparing the briquets the comminuted slag, preferably white furnace-slag, is brought into a revolving cylinder to be exposed therein in the well-known manner to a quick and thorough action of high-pressure steam. 80 The said rotatory motion may be produced by any suitable means. After permitting the steam to act as long as may be necessary upon the slag it is withdrawn and is now a suitable binder. The binder thus obtained 85 is intimately mixed with the aforesaid refuse or rotten ore, and then the mixture is supplied to any kind of briquetting-machine. The briquets removed from the latter are 90 most suitable for smelting processes. The desired degree of hardness will be attained by allowing the briquets to rest for some time before they are used. By applying the binder in the proportion of ten per cent. a porosity will be obtained which will permit 95 the gases in the upper portion of the furnace to diffuse through the briquet and to bring about the desired chemical changes. The briquet obtained in this manner is physically different from the briquet agglomerated by the fusion of slag, inasmuch as only a hydraulic binding holds the particles together sufficiently to stand handling and transportation. The binding by fusion is obtained later in the high furnace itself, where the heat destroys 100 the hydraulic binding and substitutes for it

the binding by fusion. Thus a great advantage is obtained. All the fuel spent in the manufacture of ordinary ore briquets is saved, and in the melting zone of the furnace 5 the briquets, being fritted together in the upper zones, preserve their shape, as well as the porosity.

My process can be used for briquetting any kind of ores or any waste or refuse containing 10 iron or copper or any other kind of metal.

I am aware that it has been proposed to construct a building block or stone employing a binder similar to that employed by me, but in different proportion and for an entirely 15 different purpose. My briquet is not so hard as a building-stone. If it were, its efficiency would be lost. The amount of binder is small compared with the other elements, being only sufficient to enable the 20 briquets to be handled without breaking, but sufficient to cause them to retain their shape

and porosity when in use and prevent their falling into powder.

What I claim as my invention, and desire to protect by United States Letters Patent, 25 is—

1. A porous briquet suitable for melting furnaces composed of finely-divided metaliferous material, and hydraulic slag cement, substantially as described. 30

2. A porous briquet suitable for melting furnaces composed of finely-divided metaliferous material, ten parts, and hydraulic slag cement, one part, substantially as described. 35

In testimony whereof I have hereunto signed my name in the presence of two witnesses.

HUGO SCHULTE-STEINBERG.

Witnesses:

WILLIAM ESSENWEIN,  
PETER LIEBER.